

## UNITED STATES PATENT OFFICE

2,019,899

## MOTOR FUELS CONTAINING INHIBITORS

Herbert G. M. Fischer, Westfield, and Clifford E. Gustafson, Elizabeth, N. J., assignors to Gasoline Antioxidant Company

No Drawing. Application June 10, 1933,  
Serial No. 675,399

## 6 Claims. (Cl. 44—9)

The present invention relates to improvements in low-boiling, non-viscous hydrocarbon oils, such as naphtha and the like, and will be fully understood from the following description.

5 Hydrocarbon oils, such as naphtha, which includes gasoline, and particularly such naphthas as are made by decomposition of heavier oils and the like, often contain gum or gum-forming constituents which are objectionable in many respects. The exact nature of these objectionable 10 impurities is at present unknown, but the gum content, or, more properly, gum formation tendency, is measured by the method Number 530.1 in the United States Bureau of Mines, Technical Report 323-B, entitled "Specification for Petroleum Products and Methods of Testing", revised October 21, 1927, page 96. In brief, this method 15 consists in placing 100 cc. of the naphtha to be tested in a 3½" diameter spun copper dish on a steam bath and evaporating off the volatile material. The result is expressed in milligrams of gum left in the dish per 100 cc. of the naphtha. Another method for determining the 20 tendency of products of this type to form gum is known as the breakdown method, which measures the resistance of a gasoline to oxidation as follows: A given quantity of gasoline is placed at atmospheric temperature into a suitable bomb which is connected to a pressure gauge of either 25 indicating or recording type. After the bomb is tightly closed, oxygen is allowed to flow into the bomb until a pressure of 100#/sq. in. is recorded. The oxygen supply is then shut off and disconnected. The bomb and its contents are then 30 heated in a suitable bath to a temperature of 100° C. Upon heating, the pressure will rapidly rise to a maximum (say 125#) and remain at this point until active oxygen absorption by the gasoline takes place, when a more or less rapid drop in pressure will be noted.

35 The resistance to oxidation of the gasoline is numerically expressed in minutes and is taken as the time elapsed from the application of heat until

40 Base stock used: Non-acid treated soda-washed cracked stock

til a drop in pressure of 2# below maximum is recorded. This period is generally called the induction period, at the end of which it will generally be found that the gasoline will contain between 20-30 mg. of gum as measured by the 5 preformed gum test.

As noted above, cracked naphthas containing relatively large quantities of gum are objectionable, particularly for motor fuels, cleaning naphthas, light solvents, and the like. It is also well known that on standing the gum content of many naphthas steadily increases. We have discovered 10 that the addition of mixtures of certain organic materials to the naphtha, even though in very small quantities, greatly reduces the gum as indicated by the above described tests and also prevents an increase of gum for prolonged, if not indefinite, periods.

15 We have observed that mixtures of certain derivatives of polycyclic compounds, such as naphthalene, anthracene and phenanthrene, are useful for our purpose. The substitution of certain groups in the alpha position greatly increases the 20 effect of the addition agents, for example, we have observed that mixtures of agents such as alpha naphthol and alpha naphthylamine may be added to the gasoline with good results and that volatile metallic compounds, such as metallo-organic substances, which are useful for 25 their anti-detonating effects, may be present in 30 the naphthas without any adverse action.

35 The quantity of the addition agents is very small, not being greater in any case than 5 gr. per liter of the naphtha and generally between the approximate limits of .01 to 1.0 gr. per liter. There appears to be an optimum quantity of the 40 agents which will give the best results and it is a simple matter to make up solvents of different strengths and empirically select the most suitable concentration.

45 The following table indicates the effect obtained by adding alpha naphthol and alpha naphthylamine to cracked stock (gasoline).

| Inhibitor                                             | Copper dish gum | Induction period minutes | Gum content 1 hour after induction period Mg./100 cc. | Total heating period minutes |
|-------------------------------------------------------|-----------------|--------------------------|-------------------------------------------------------|------------------------------|
| Base stock                                            | 79              | 65                       | 288                                                   | 125 50                       |
| None                                                  | 12              | 110                      | 268                                                   | 170                          |
| +.006% alpha naphthol                                 | 10              | 145                      | 282                                                   | 205                          |
| +.01% alpha naphthol                                  | 25              | 80                       | 138                                                   | 140                          |
| +.006 alpha naphthylamine                             | 71              | 90                       | 140                                                   | 150                          |
| +.01% alpha naphthylamine                             | 20              | 95                       | 152                                                   | 155                          |
| +.0025% alpha naphthol and .0025% alpha naphthylamine | 13              | 125                      | 112                                                   | 185                          |
| +.005% alpha naphthol and .005% alpha naphthylamine   |                 |                          |                                                       |                              |

The term "naphthalene compounds" having certain substituted groups, is used in this specification to include the substituted naphthalene itself, the substituted homologues and the derivatives thereof.

The explanation for the enhanced gum inhibiting effect of the mixed antioxidants is believed to be that the combined action of these anti-oxidants or naphthalene compounds having certain substituted groups prolong the induction period of the treated naphtha and further retard the formation of gum after the induction period. It should be understood that our invention is not to be limited by any theory of the mechanism of the process nor by any example given merely by way of illustration, but only by the following claims in which we wish to claim all novelty inherent in the invention.

This application is a continuation in part of our copending application 307,545 filed September 21, 1928.

We claim:

1. The method of inhibiting the formation of gum in cracked gasoline, which comprises adding to said gasoline a small proportion of a mixture of anti-oxidants comprising alpha-substituted aromatic condensed ring hydrocarbons in which adjacent nuclei have two carbon atoms in common, some of said hydrocarbons having an amino substituent and others an hydroxy substituent.

2. As a composition of matter a low boiling hydrocarbon oil prepared by heat treatment at a decomposition temperature and normally tending to form gum, and a small proportion of a

mixture of anti-oxidants comprising alpha substituted aromatic condensed ring hydrocarbons in which adjacent nuclei have two carbon atoms in common, some of said hydrocarbons having an amino substituent and other an hydroxy substituent.

3. The method of inhibiting the formation of gum in cracked gasoline, which comprises adding to said gasoline a small proportion of a mixture of anti-oxidants comprising a substance having the characteristics of alpha naphthol and a substance having the characteristics of alpha naphthylamine.

4. As a composition of matter a low boiling hydrocarbon oil prepared by heat treatment at a decomposition temperature and normally tending to form gum, and a small proportion of a mixture of anti-oxidants comprising a substance having the characteristics of alpha naphthol and a substance having the characteristics of alpha naphthylamine.

5. The method of inhibiting the formation of gum in cracked gasoline, which comprises adding to said gasoline a mixture of antioxidants comprising alphanaphthol and alphanaphthyl-25 amine.

6. As a composition of matter a low boiling hydrocarbon oil prepared by heat treatment at a decomposition temperature and normally tending to form gum and a small proportion of a mixture of antioxidants consisting of alphanaphthol and alphanaphthylamine.

HERBERT G. M. FISCHER.  
CLIFFORD E. GUSTAFSON. 35